

May 26, 1925.

H. FISH

1,539,413

LATHE CENTERING TOOL

Filed Jan. 10, 1923

Fig:1.



Fig:3.



Fig:6.



Fig:2.



Fig:4.



Fig:7.



INVENTOR

5 Harold Fish

BY *Mock & Blum*  
ATTORNEYS

## UNITED STATES PATENT OFFICE.

HAROLD FISH, OF BRIDGEPORT, CONNECTICUT.

## LATHE CENTERING TOOL.

Application filed January 10, 1923. Serial No. 611,883.

*To all whom it may concern:*

Be it known that I, HAROLD FISH, a citizen of the United States, residing at Bridgeport, in the county of Fairfield and State of Connecticut, have invented certain new and useful Improvements in Lathe Centering Tools, of which the following is a specification.

My invention relates to a new and improved tool and method of making the same.

One of the objects of my invention is to provide a new and improved construction for high speed steel cutting lathe tools and the like.

Another object of my invention is to provide a new and improved tool in which the working part, made of high speed steel or stellite or the like, is inserted into a holder made of another material, such as a cheap machine steel.

Another object of my invention is to provide a combination tool in which an operating portion is inserted into a holding portion, and in which the said operating portion is held very firmly in the said holding portion.

Other objects of my invention will be set forth in the following description and drawings which illustrate a preferred embodiment thereof.

Fig. 1 is an elevation of the holder of my tool.

Fig. 2 is a section on the line 2—2 of Fig. 1.

Fig. 3 is an elevation of the operating portion of my tool.

Fig. 4 is a section on the line 4—4 of Fig. 3.

Fig. 5 is an elevation showing a completely assembled tool.

Fig. 6 is a view similar to Fig. 5 but is partially in vertical section.

Fig. 7 is a section on the line 7—7 of Fig. 6.

The holder is made of any suitable material such as a cheap machine steel. As clearly shown in Fig. 6, this is drilled so as to provide a recess 2 which extends for about half the length thereof. After the drilling

of the recess 2 has been completed, it is reamed so as to cause the wall thereof to have a slight taper, namely about 7°. The wider part of the said recess 2, after the reaming thereof to bring the desired taper, is at the frustro-conical tip 3 of the said

holder 1. It will be noted that the inner end 4 of the recess 2 has a conical contour.

A piece of stellite or high speed steel 5 is then taken and a piece of cheap machine steel or the like 6 is welded to the blunt end thereof. The member 5 is also provided with a conical point 7 which has preferably the same angle as the frustro-conical tip 3 of the holder 1. The combination piece formed by the cutting member 5 and the end member 6 is then turned and ground to exactly the same taper as the holder or recess 2 in the shank 1, so that if the cutting member were driven into the said shank, what is called a "drive" fit would be produced and it would be practically impossible to get it out.

I prefer, however, to first put the shank or holder 1 into a low heat furnace and bring it up to the proper temperature, namely about 800° or 900° F. so as to produce a shrink fit. The cutting member which is cold and has been properly hardened, is powerfully pressed or forced into the correspondingly tapered hole 2. The hot shank is then quenched by any suitable method, so as to cause it to rapidly shrink and a perfect joint or union between the shank and the cutting member is thus produced. It will be noted that when the tapered cutting member is powerfully forced into the tapered hole 2, that it does not distort the holder adjacent the conical portion 4 of the hole 2.

I have shown a preferred embodiment of my invention but it is clear that numerous changes and omissions can be made without departing from its spirit.

When the relatively cold tool is forced into the hole 2, which has been enlarged by the heat, the cold walls of the tool are powerfully forced against the hotter interior walls of the shank which are at about 800° F. as before mentioned. This causes an immediate chilling of the interior wall of the shank tube which is followed by the rapid chilling of the entire body of the shank when the quenching operation is performed.

The ordinary machine steel previously mentioned herein is a carbon steel. It is important to heat the shank or holder 1, made of this carbon steel to a temperature of between 800° to 900° F. because if a lower temperature is employed then the correct shrink is not secured when the hot

shank is quenched in water, and if a higher temperature is employed then when the cutting member is powerfully pressed therein, the shank or body is distorted thus making it 5 useless.

I claim:—

1. A method of making a tool consisting of an operating member having a tapered rear end held in a shank having a correspondingly tapered recess, which consists in heating the shank, then forcing the tapered end of the operating member into the recess of the heated shank with strong longitudinal pressure, and then cooling the shank, the 10 said longitudinal pressure being sufficient and the said temperature being such that the operating member is held in the shank without any relative movement between them.
2. A method of making a cutting tool which consists in forming a shank made of machine steel with an outwardly tapering hole therein, heating the said shank so as 15 to enlarge the said hole, driving into the said

hole a correspondingly tapered cutting member 25 and then quenching the said shank, the temperature of said shank after the heating thereof being sufficiently high to cause the shrinkage thereof upon quenching to tightly bind said cutting member in said shank, said 30 temperature being sufficiently low to avoid any distortion of the parts when said cutting member is forced into said shank.

3. A tool comprising a metal shank having a tapered recess therein having an inclined wall, and an operating member having a correspondingly tapered end fitting in said recess, the said shank having the metal wall of said recess being in tight contact 35 with said tapered end and being compressed 40 in a direction perpendicular to said wall, the said shank being shrunk about said tapered end, the said tapered end being in such tight contact with the wall of said recess to prevent any relative movement. 45

In testimony whereof I hereunto affix my signature.

HAROLD FISH.